

## UNITED STATES PATENT OFFICE.

ADOLPHE EUGÈNE MARIE ROUSSEAU, OF PARIS, FRANCE

## METHOD OF TREATING VEGETABLE TEXTILE FIBERS

No. 909,457.

Specification of Letters Patent.

Patented Jan. 12, 1908.

Application filed October 19, 1906. Serial No. 339,706.

*To all whom it may concern:*

Be it known that I, ADOLPHE EUGÈNE MARIE ROUSSEAU, of Paris, France, have invented a certain new and useful Method of Treating Vegetable Textile Fibers, which invention is fully set forth in the following specification.

After the operation of stripping or scutching, which has the result of separating the stalk or ligneous bark which surrounds the filaments of flax and hemp which are thereby brought to the condition of tow, these filaments are still surrounded by a resinous and colored substance from which they are freed by a series of lixiviating and bleaching operations.

In the processes hitherto adopted lixiviating with soda or other alkaline reagents precedes the chlorinating, that is to say the bleaching with the decoloring chlorids.

The principle of this invention consists broadly in inverting the order of these operations and in beginning with the bleaching and in then subjecting the textile fibers to a series of operations the object of which is to further bleach them and render them more silky and of a high degree of tenuity, in keeping them ready to be subjected to the operation of combing and then to that of spinning under the best conditions.

The inventor has been led to devise this novel process by noticing that if textile fibers are bleached before ungumming them by means of the lye, the decoloration and the bleaching are effected equally well and present the advantage of refining and bleaching the gummy or resinous substances which surround the fiber, and which may thus be collected and placed on the market without further treatment for the purposes for which these materials may be adapted. Having explained this, the operations which constitute the novel process will now be described, in indicating the composition of the baths in which the fibers to be treated should be immersed successively.

1. The first operation, as stated above, is the bleaching. Preferably a bath having a base of decoloring chlorid composed in the following manner is employed:—In 100 liters of water at the ordinary temperature of the open air, about 5 liters of a liquid having a density of 0.907 is added, this liquid being obtained by dissolving: (a) 10 kgs. of chlo-

Ca(OCl)<sub>2</sub>, CaCl<sub>2</sub>, and CaCO<sub>3</sub>, in 120 liters of water. (b) 12 kgs. of carbonate of potash K<sub>2</sub>CO<sub>3</sub>, dissolved in 40 liters of water at 100°. These two solutions (a) and (b) are combined and form the bath in which the textile fibers in the condition of tow, flax, hemp, ramie, etc., are steeped, leaving them there until the appearance of bleaching is noticeable. Instead of a chlorin bath, oxygenated water or ozone may be employed as decoloring agent. The inventor has found that the decoloring action penetrates as far as the fiber and is at the same time exerted upon the gummy or resinous portion which surrounds it.

2. The textile fibers thus bleached are then immersed in another receptacle containing a bath of water to which has been added: (c) sulfite of soda (SO<sub>3</sub>Na<sub>2</sub>, 10 H<sub>2</sub>O) in sufficient quantity for neutralizing the action of the first bath; and 30% of the weight of the textile tow to be treated of a compound obtained in accordance with the following formula:—(d) 30 kgs. of a soap formed of 28 parts of margarin, 72 parts of olein combined with 4 kgs. of carbonate of soda Na<sub>2</sub>CO<sub>3</sub> and 45.5 kgs. of water. In order to obviate the repetition of this long chemical formula, which will again be employed, the soap which it represents is hereinafter designated by the letter S. The temperature of this grease-removing bath so composed is that of the surrounding atmosphere. The duration of the immersion of the textiles in this bath is about 1 hour.

3. A fresh elimination of grease is then effected, this time with the employment of heat in a bath composed of water to which is added the said soap S in the proportion of 50% of the weight of the textile treated. The temperature of the bath is raised progressively to a temperature of from 90° to 95° C. It is maintained at this temperature for a period of 2 to 4 hours. After this operation the fibers are subjected to a second rinsing in clean water which is at first hot.

4. The succeeding operation is properly speaking the ungumming operation, the result of which is to free the fibers from their gummy or resinous covering, which, being insoluble, has not been removed by the preceding operations. The ungumming bath is composed of water to which there are added: (f) The said soap S in the proportion of 3% of the textile. (g) Bi-sulfite of soda (NaHSO<sub>3</sub>), 3% of the textile. (h) Car-

bonate of soda  $\text{Na}_2\text{CO}_3$ , 2% of the textile. The temperature of the bath is the surrounding temperature and the duration of the immersion there is from two to four hours. It is followed by a third rinsing in water.

5. The treatment is completed by immersing the textile fibers in a bath of water, to which there is added:—(i) Amylactic ether in the proportion of 1% of the textile. The 10 immersion takes place at the surrounding temperature and should last for two hours. The effect of the amylactic ether is to impart to the textile fibers a luster or brilliancy, which makes them silky, and to render soluble the last insoluble portions of the resinous coating. On leaving this bath the material is rinsed in cold water at the surrounding temperature.

20 After these various operations, the drained textile fibers are placed to dry, in the open air if possible. When once it is dry, the textile is ready for combing and it furnishes exceedingly white fibers, which are silky and of great strength, so that it is possible to 25 obtain the finest threads immediately in spinning, the count 200 for example and be-

yond, with a greater yield and an economy of time and a reduction in the cost price hitherto unattainable.

What I claim is—

The process of treating vegetable fibers such as flax, hemp, ramie and the like to bleach and remove the gummy and resinous coating surrounding the fibers, consisting in bleaching the gummy and resinous coating 30 surrounding the fibers by means of a bleaching bath; neutralizing the bleaching agent adhering to the fibers after bleaching, by means of a sulfite-containing soap; subjecting the fibers so treated to a soap bath; then 40 to an ungumming bath containing hyposulfite of soda, an alkali carbonate and soap; and finally to an aqueous bath containing amylactic ether.

In witness whereof I have hereunto signed 45 my name this 4th day of October 1906, in the presence of two subscribing witnesses.

ADOLPHE EUGÈNE MARIE ROUSSEAU.

Witnesses:

HANSON C. COXE,  
GABRIEL BELLARD.